# EUROPEAN PATENT SPECIFICATION

(11) **EP 0 005 873 B1**
(45) Date of publication and mention of the grant of the patent: **23.06.1982**
(21) Application number: 79200228.9
(22) Date of filing: 10.05.1979
(51) Int. Cl.: C10M 1/26, C07C 69/52

(54) **A liquid hydrocarbon oil composition containing an ester of an unsaturated carboxylic acid**
Eine flüssige Kohlenwasserstoffölverbindung, die einen Ester einer ungesättigten Carbonsäure enthält
Composition d'huile d'hydrocarbure liquide contenant un ester d'un acide carboxylique insaturé

(30) Priority: 22.05.1978 GB 2104978
(43) Date of publication of application: 12.12.1979
(73) Proprietor: SHELL INTERNATIONALE RESEARCH MAATSCHAPPIJ B.V., 2596 HR Den Haag (NL)
(72) Inventor: Berger, Hans, NL-1031 CM Amsterdam (NL)
(74) Representative: Puister, Antonius Tonnis, Mr.

## Description

The invention is concerned with hydrocracked lubricating oil compositions having improved resistance against the formation therein of insoluble material.

From British patent 442,921 it is known to improve the oiliness of hydrocarbon lubricating oils, which may have been refined by destructive hydrogenation, by adding a minor proportion of an ester of an alcohol containing at least 10 carbon atoms and e.g. an unsaturated carboxylic acid with less than 4 or 5 carbon atoms.

It has now been found that a special class of such esters reduce the amount of insoluble material formed in hydrocracked lubricating oils, which normally tend to form insoluble material during use especially at high temperatures e.g. at temperature of at least 100°C.

Accordingly, the invention is concerned with a hydrocracked lubricating oil composition comprising 0.001 to 10%w of an ester of an olefinically unsaturated carboxylic acid and a C₁₀ to C₃₀ alkyl alcohol, characterized in that the ester is an ester of acrylic and/or methacrylic acid.

The esters may be prepared by any suitable technique such as by transesterification but are suitably prepared by direct esterification of the appropriate acid with the appropriate alcohol. Suitable alcohols include linear or branched and primary, secondary or tertiary alcohols. A single alcohol or a mixture of alcohols may be used. The alcohols may be natural or synthetic e.g. hydroformylation alcohols.

In general, hydrocracking is a severe hydrogenation treatment under conditions which depend upon the nature of the oil but usually comprises contacting the feedstock with hydrogen in the presence of a hydrogenation catalyst at a temperature usually between 350 and 500°C and at a pressure usually between 60 and 200 bars. Hydrocracking is usually performed in place of a conventional solvent extraction step. Hydrocracking usually increases the viscosity index of the feed-stock and is used in the preparation of high, very high and extra high viscosity index lubricating oils. The hydrocracked lubricating oils may also be subjected to a hydrofinishing step which is a mild hydrogenation step.

The amount of ester may vary between wide limits from 0.001. to 10%w, preferably from 0.01 to 2.0%w, based on the weight of the hydrocarbon oil.

The lubricating oil composition may contain other additives such as pour-point depressants, anti-corrosion agents, additives to improve the viscosity and viscosity-temperature characteristics, anti-oxidants, metal passivators, extreme pressure and anti-wear additives.

The invention will now be illustrated by the following examples.

### Examples 1 and 2

In these Examples a liquid hydrocracked hydrocarbon lubricating oil was used which was derived from a crude mineral oil. The lubricating oil has a VI of 94.5 and a viscosity (98.9°C) of 5.11×10⁻⁶ m²/s (5.1 centistokes). To the lubricating oil was added 1%w of either a C₂₀/C₂₂ (1:4) alkyl acrylate (Example 1) or a C₂₀/C₂₂ (1:4) alkyl methacrylate (Example 2). The oil composition (30 g) and the oil itself (30 g; Example a; comparative) were tested by blowing air through the mixture (15 litres/hour) for 168 hours after which the amount of insoluble material formed was determined. The results obtained were 0.36%w (Example 1), 0.33%w (Example 2) and 0.55%w (Example a).

## Claims

A hydrocracked lubricating oil composition comprising 0.001 to 10%w of an ester of an olefinically unsaturated carboxylic acid and a C₁₀ to C₃₀ alkyl alcohol, characterized in that the ester is an ester of acrylic and/or methacrylic acid.

## Revendications

Ein hydrogecrackte Schmierölmischung ent- haltend 0,001 bis 10 Gewichtsprozent eines Esters von einer olefinisch ungesattigten Carbonsaüre mit einem C₁₀ bis C₃₀ Alkyl- alkohol, dadurch gekennzeichnet, dass der Ester ein Ester von Acryl- und/oder Methacrylsaüre ist.

## Patentansprüche

Composition d'huile lubrifiante d'hydro- craquage comprenant de 0,001 1 10% en poids d'un ester d'un acide carboxylique olefiniquement non sature et d'un alcool alcoylique de C₁₀ ä C₃₀, caractérisée en ce que l'ester est un ester d'acide acrylique et/ou d'acide mäthacrylique.
